

## UNITED STATES PATENT OFFICE

2,238,771

## PENCIL LEAD

Isidor Chesler, Oceanport, N. J., assignor to Eagle  
Pencil Company Inc., New York, N. Y., a cor-  
poration of Delaware

No Drawing. Application December 30, 1939,  
Serial No. 311,944

15 Claims. (Cl. 120—83)

The present invention relates to a pencil lead which makes a mark of conventional appearance, capable of being readily identified as having been made by the lead of this invention rather than by an ordinary lead.

In the classification of cards or papers by that type of statistical machine which records pencil marks of low electrical resistance, a negative registration would result, if through carelessness, inadvertence or design the markings were made with an ordinary pencil. The invention in one particular application is accordingly intended to render possible the ready verification of the use of such specialized pencil lead.

Among the objects of the invention are to provide a pencil lead that has the required characteristics, such as low electrical resistance of the mark made thereby and that affords a distinctive tell-tale indication upon appropriate test, without sacrifice of the various desirable properties of known leads of good quality, including durability, uniformity, and smooth writing of predetermined hardness or softness.

Another object is to provide a lead of the above type, the cost of production of which is but slightly higher than that of ordinary leads of corresponding quality and which is not subject to deterioration in any respect even long after it has been fabricated.

Another object is to provide a lead of the above type which, despite its specialized properties, has no ingredients therein apt to impair or destroy the card or paper on which the pencil is used and which has no toxic constituent apt to cause injury by contact with the fingers or tongue of the user.

According to the invention, the lead prepared of one of the usual mixtures of graphite and clay, fired according to conventional practice, has incorporated in the minute interstices thus formed therein and prior to wax or oil impregnation thereof, some color agency either in the form of a suitable soluble dye, or of a dye intermediate or an indicator that gives a color reaction upon appropriate treatment, so that when a pencil marking on the sheet is suitably moistened, a tell-tale coloration will appear, where an ordinary lead pencil mark would show no change upon corresponding treatment.

It is preferred to use as the color medium a dye, such as rhodamine, eosine, methylene blue or methyl violet. A solution of the dye will readily penetrate into the interstices of the fired lead. It is advantageous to impregnate the leads with a solution of such dye in a relatively

5 volatile solvent such for instance as alcohol. After such impregnation, the leads are drained and then dried by tumbling in sawdust. Thereupon, the alcohol solvent would be evaporated by placing the leads in an oven at a suitable temperature for a sufficient period of time. As a consequence, the dry dye will remain as a deposit on the walls of the labyrinthine interstices or pores. The leads are thereupon preferably impregnated with further dye in a non-volatile hygroscopic solution, then drained, rinsed and dried. Finally the leads are desirably impregnated in oil or wax and tumbled in sawdust.

15 In one specific way of carrying out the invention, the leads prior to wax or oil impregnation thereof, are immersed in a bath of a volatile carrier such as ethyl alcohol containing five per cent by weight of a dye such as rhodamine. To insure solution of the dye, the bath is first heated and the immersion may be at room temperature, desirably for about three hours. The leads are then removed from the bath, drained, dried in sawdust and spread on a screen overnight at room temperature to allow complete evaporation of 20 the alcohol from the leads.

25 After the leads have thus been dried, they are immersed in a second bath including preferably a non-volatile carrier comprising a solution of a hygroscopic polyhydric alcohol such as glycerin 30 with associated water, an ionogen such as boric acid and a dye such as rhodamine in suitable proportions. Desirably, the ingredients of the second bath are in the proportion of 200 c. c. of glycerine to 75 grams of boric acid and 7.5 35 grams of rhodamine. The bath is kept at a temperature of about 120 degrees C. and the leads remain immersed therein for about three hours. Thereafter, the leads are removed and drained for not more than a couple of minutes and thereupon quickly rinsed in cold water and dried in 40 sawdust.

45 Finally the leads are impregnated with oil or grease according to usual practice, but it is preferred for the particular purpose in hand to immerse them for about fifteen minutes in tallow kept at 110 degrees C., the excess being thereupon cleaned off by tumbling in sawdust.

50 The lead of the specifications set forth will maintain its efficacy for long periods of time, by reason of the fact that the hygroscopic glycerin ingredient thereof retains sufficient water to maintain the boric acid and the dye in solution therein at all times and the tallow acts to a large extent as a seal to keep the water retained by the glycerine from escaping with rise in tem-

perature and to preclude excess water from entering under conditions of excessive humidity.

Even though the mark made by the lead is not fresh, it will have all the properties required for the present purpose. The mark will be black and of the desired degree of hardness. The glycerin-water ingredient of the mark will have in solution therein both the boric acid and the dye and the water is kept in situ by the tallow, so that the electrical resistance of the mark is and remains low as required for the particular specific purpose for which the lead is adapted.

Lead prepared in the manner set forth will give a black mark indistinguishable to the eye from that made by ordinary lead pencils of corresponding grade and quality. To test the mark in order to verify whether it has been made with the specialized pencil, a drop of alcohol need merely be applied to a portion of the mark. It immediately dissolves some of the rhodamine and leaves a halo about the mark as the drop spreads, giving the tell-tale indication which is lacking when alcohol is applied to a mark made by an ordinary pencil.

While ethyl alcohol pure or denatured is preferred as the solvent, it is obvious that other solvents such as methyl alcohol may be used, but by reason of the toxic character of some of such other solvents, the ethyl alcohol is to be preferred.

Another way of producing substantially the identical lead above described is by immersing the fired leads in a concentrated boiling solution of the soluble dye and after drying impregnating the leads in the oleaginous material set forth.

Instead of alcohol soluble dyes such as those above suggested, an oil soluble dye might be used, such as double xylylidine compound for red. The use of such oil soluble dye has the advantage that it could be admixed with the waxes or oils employed and the mixture could be applied in a single impregnation. With such dyes the paper would be moistened at a marked area with an oil solvent, preferably a hydrocarbon such for instance as benzine, in order to test for the tell-tale indication.

Instead of a dye, a suitable dye intermediate could be used, and a marked area would be moistened with an appropriate developer to test for the tell-tale trace.

Another alternative is an indicator such as phenolphthalein, desirably in a glycerin carrier, preferably with about ten per cent of the indicator dispersed therein. The leads would be immersed in the glycerin mixture for about fifteen minutes at a temperature of about 285 degrees C. and after removal from the mixture would be rinsed in cold water for fifteen minutes and thereupon dried in sawdust. For verifying the identity of a mark made with a lead thus impregnated a marked area would preferably be wetted with a weak alkaline solution to test for a tell-tale red mark.

Where the leads are to be used with a statistical machine of the type that depends on low electrical resistance of the pencil mark, it is desirable to use in the lead a graphite of relatively low resistance.

The invention is not limited in its application to leads that make such low resistance mark as is required for use with statistical machines of the type referred to. An ordinary fired lead when subjected to the treatment, above set forth, might be useful for instance for facilitating detection of alterations in a pencil document written with the special lead.

As many changes could be made in the above

article and method and many apparently widely different embodiments of this invention could be made without departing from the scope of the claims, it is intended that all matter contained in the above description shall be interpreted as illustrative and not in a limiting sense.

Having thus described my invention, what I claim as new and desire to secure by Letters Patent is:

10. A pencil lead of fired graphite and clay having a soluble colored ingredient lodged in the pores thereof, ineffective to alter the black coloration of the mark made by the lead and upon the application of a suitable liquid to yield a tell-tale indication in the form of a halo of contrasting color.
15. A pencil lead of fired graphite and clay having a colored ingredient lodged in the pores thereof, ineffective to alter the black coloration of the mark made by the lead and upon the application to such mark of a suitable solvent for the colored ingredient to yield a tell-tale trace in the form of a halo of contrasting color.
20. A pencil lead of fired graphite and clay having dye lodged in relatively dry condition in the pores thereof, ineffective to alter the black coloration of the mark made by the lead and upon the application to such mark of a solvent for the dye yielding a tell-tale indication in the form of a halo of contrasting color.
25. A pencil lead of fired graphite and clay having deposited in the pores thereof, a dye of the group which consists of eosine, rhodamine, methylene blue and methyl violet, said dye being ineffective to alter the black coloration of the mark made by the lead and upon the application to the mark of a drop of dye solvent yielding a tell-tale indication in the form of a halo of contrasting color.
30. A pencil lead of fired graphite and clay having the pores thereof substantially filled with a waxy substance and an oil soluble dye ineffective to alter the black coloration of the mark made by the lead and soluble upon the application to such mark of suitable solvent, to yield a tell-tale indication in the form of a halo of contrasting color.
35. A pencil lead of fired graphite and clay having the interstices thereof impregnated with a non-volatile liquid ingredient of hygroscopic character having in solution therein an ionogen and a dye.
40. A pencil lead of fired graphite and clay having the interstices thereof filled with water carrying glycerin, boric acid, rhodamine dye and tallow.
45. A pencil lead of fired graphite and clay having the interstices thereof impregnated with a polyhydric alcohol of hygroscopic character having in solution therein an ionogen and a dye soluble in the polyhydric alcohol.
50. A pencil lead of fired graphite and clay having the interstices thereof filled with water carrying glycerin, boric acid, rhodamine dye and tallow.
55. A pencil lead of fired graphite and clay having the interstices thereof impregnated with a chemical indicator in a non-aqueous carrier.
60. A pencil lead of fired graphite and clay having the interstices thereof impregnated with phenolphthalein in glycerin.
65. The method of preparing a pencil lead the mark of which will show a contrasting color when treated with appropriate liquid, which comprises impregnating the fired lead with a hygroscopic non-volatile liquid carrier having an ionogen and a dye in solution therein.
70. The method of preparing a pencil lead the mark of which will show a contrasting color
75. The method of preparing a pencil lead the

when treated with appropriate liquid, which comprises impregnating the fired lead with a volatile carrier having coloring matter distributed therein, evaporating the carrier and thereupon impregnating the lead with a non-volatile hygroscopic carrier having an ionogen and a dye in solution therein.

13. The method of preparing a pencil lead the mark of which will show a contrasting color when treated with appropriate liquid, which comprises impregnating the fired lead with glycerin having boric acid and a dye in solution therein.

14. The method of preparing a pencil lead the

mark of which will show a contrasting color when treated with appropriate liquid, which comprises impregnating the fired lead with a volatile carrier having dye in solution therein, evaporating the carrier therefrom, then impregnating the lead with a non-volatile hygroscopic carrier having an ionogen and dye dissolved therein and finally impregnating the lead in an oleaginous bath.

15. The method recited in claim 14 in which the non-volatile hygroscopic carrier is glycerin and the ionogen is boric acid.

ISIDOR CHESLER.